

Dec. 10, 1929.

S. RUBEN

1,739,044

METHOD OF TREATING ELECTRON EMISSION ELEMENTS

Filed Jan. 12, 1927



Inventor  
Samuel Ruben

By his Attorney McClellan

## UNITED STATES PATENT OFFICE

SAMUEL RUBEN, OF NEW YORK, N. Y., ASSIGNOR TO RUBEN TUBE COMPANY, A CORPORATION OF DELAWARE

## METHOD OF TREATING ELECTRON-EMISSION ELEMENTS

Application filed January 12, 1927. Serial No. 160,758.

This invention relates to a method of treating electron emission elements, and more particularly it relates to a method of treating cathode elements by coating them with a dense 5 layer of alkaline earth oxides to increase the electron emission beyond that of the metal bases used as cathodes in electron emission devices.

In the prior art the metal cathodes have 10 had their emission characteristics increased by coatings of alkaline earth oxides by (1) applying to the cathode base an oxide mixture, or a single oxide, with a binder material, which latter is then carbonized or vaporized off, (2) applying an oxide with another compound and decomposing the latter to allow to remain an adherent residue of the desired oxide and, in some instances, a portion 15 of the binder element in the form of a finely 20 divided metal and (3) passing the cathode base through a molten mixture of oxides.

While such treatment temporarily improves the cathode emission, for adequate service these coatings lack uniform distribution, proper density and permanent electrical contact with the base, causing excessive 25 resistance losses in the coating material. At higher voltages a strong electrostatic attraction away from the cathode to the anode 30 carries the coating particles with it.

I have found that by applying a coating of alkaline earth oxide material of high emissivity, such as strontium or barium, to the surface of the cathode element and, after 35 drying the coating and driving off the binder element, heating the coating material to a point just below its melting temperature and compressing it, there remains an oxide coating that is dense, uniformly distributed and of 40 low electrical resistance, and having a life and efficiency greatly above that obtained from coatings treated by the former methods. By this treatment the oxide particles being 45 held in a compact mass and closely adherent to the metal base surface, the tendency towards disintegration of the coating material is greatly diminished.

For a better understanding of the invention, reference is made to the accompanying 50 drawing diagrammatically illustrating an ap-

paratus by which the method of application and treatment of coating by my invention may be followed, in which, 1 represents a tungsten wire cathode in process of being passed by spools 3, 3<sub>a</sub> and 3<sub>b</sub>, through solution 2 of strontium and barium oxides mixed with gum arabic, over heated dryer 4, supplied with energy by generator 6, between heated rolls 5 under compression and on to a reel. As the wire passes over heated dryer 3, the binder 55 element is driven off and the oxide coated wire is carried to compression rolls with the oxide coating at approximately the melting temperature of the oxides, the rollers compressing the coating mass and making it more dense and 60 adherent to the metal base, and therefore giving the cathode element a higher degree of 65 emissivity and longer life.

What I claim is:

1. The method of treating an electron emission element which consists in applying a mixture of an alkaline earth oxide and a binder material to the surface of the element, heating the coating layer on the element and compressing the coating layer at a temper- 70 75

ature close to its melting temperature. 2. The method of treating an electron emission element which consists in applying a mixture of alkaline earth oxides and a binder material to the surface of the element, heat- 80 85

ing the applied mixture on the element and compressing the coating of the element at a temperature below the melting temperature of the coating mixture of oxides. 3. The method of treating an electron emission element which consists in applying to the surface of the element a mixture of strontium and barium oxides with a binder material, heating the coated element and compressing the applied coating of oxides while 90 95

heated to a plastic condition. 4. The method of treating an electron emission element which consists in immersing the element in a mixture of strontium and barium oxides with a binder material, with- 100

5. The method of treating an electron emission element which consists in applying a mixture of an alkaline earth oxide to the surface of the element, heating the coating layer on the element and compressing the coating layer at a temperature close to its melting temperature.

5  
10 In testimony whereof, SAMUEL RUBEN has signed his name to this specification this tenth day of January, 1927.

**SAMUEL RUBEN.**

**15**

**20**

**25**

**30**

**35**

**40**

**45**

**50**

**55**

**60**

**65**